

## UNITED STATES PATENT OFFICE

2,204,262

## METHOD OF PRODUCING SUEDE FINISH

Ernest Rudolf Stern, Forest Hills, N. Y., assignor  
to Sandoz Chemical Works, Inc., New York,  
N. Y., a corporation of New York

No Drawing. Application January 10, 1938,  
Serial No. 184,249

31 Claims. (CL 149—6)

This invention relates to the leather art. More particularly, it relates to a method of treating leather to produce a non-croaking suede finish which is preferably characterized by a luster or sheen and silky feel or hand comparable to genuine French antelope.

Prior to this invention French antelope was prepared by a process wherein one skin at a time was treated on a table and the manipulative steps were performed manually. Consequently, such a method and procedure required considerable time, in addition to being very tedious and uneconomical.

The instant invention overcomes the disadvantages of the prior art and provides an economical method of producing a non-croaking suede finish preferably having a luster or sheen and silky feel or hand comparable to genuine French antelope.

The instant invention further contemplates producing a non-croaking suede finish, preferably having a luster or sheen and silky feel or hand comparable to genuine French antelope, on kid, calf or sheep suede or the like by a process in which a relatively large number of skins, such as, for example, at least fifteen dozen, and preferably more, can be simultaneously treated at one time.

The instant invention further provides a method wherein the steps of appropriately coloring the skins and rendering the fibers thereof in condition for the development of the desired sheen and feel are performed in an apparatus in a relatively short period of time whereby the tedious manual operations are overcome.

Other objects of the invention will become clear and apparent from the following description and appended claims.

As is clear from the objects, one of the essential features of the invention contemplates the production of a non-croaking suede finish preferably having a luster or sheen and silky hand or feel comparable to genuine French antelope.

The suede finish contemplated by the instant invention may be provided onto tanned stock (leather) produced from kid, calf, sheep suede, splits or the like, irrespective of the tannage. Thus, the leather which is to be provided with the desired suede finish may be tanned with any of the known tannages, such as, for example, chrome tannage, aldehyde tannage, vegetable tannage, iron tannage, or any skin in which the gelatin thereof has been converted to a tanned condition. When the tannage is other than chrome tannage, the former is stripped and a chrome tannage substituted in whole or part therefor.

In accordance with the principles of the method constituting one phase of the instant invention, the selected stock which is to be provided

with a suede finish having a luster or sheen and silky feel or hand comparable to genuine French antelope is provided with a body or foundation color depending on the color desired in the final product. After the stock has been colored, it is treated to render at least the surface fibers thereof in condition so that, upon finishing, as hereafter more fully described, the luster or sheen and silky feel or hand are obtained.

Prior to or simultaneously with the treatment of the stock in order to render the surface fibers thereof in condition for producing the sheen and feel by finishing, the stock may be further dyed so as to produce the desired tinctorial effect (tone control) in the final product.

All of the aforementioned steps, except the finishing, are performed at controlled temperature conditions in an apparatus. In other words, the coloring of the stock to the desired tone and the chemical treatment of the surface fibers are effected in an apparatus under controlled temperature conditions.

In the preferred embodiment of the invention the previously mentioned steps of producing the desired tinctorial effects and converting the fibers so that the desired luster or sheen and silky feel or hand are secured upon finishing are effected in a drum under controlled temperature conditions. The drum is of any shape and of such dimensions or capacity so that the relatively large number of skins (fifteen dozen or more) which are to be treated at one working and the reagents added during the process fill only a portion of the drum, such as one-third thereof. The drum is provided with an appropriate temperature control device whereby the temperature of the contents thereof may be regulated or controlled during the process.

When the skins are given a beating action during the various stages of the process, better results are secured. The beating action of the skins may be secured in various manners. In one form of the invention this can be secured by providing the skins and the reagents employed in the various stages of the process with a relative movement with respect to each other. This can be secured by imparting a rotary, tumbling or combined rotary-tumbling, or any other movement of the drum which imparts relative movement between the materials constituting the contents thereof during the process.

When an increased beating action is desired, this can be secured by providing rubber balls in the drum. Thus, upon rotating or tumbling of the drum, the balls will also aid in beating the skins.

Another form of increasing the beating action can be secured by providing the interior surfaces of the drum with means, such as, for example, pegs or narrow shelves, disposed at spaced in-

5 tervals. In this construction, upon rotation or tumbling of the drum, the goods are alternately removed from the solution and then dropped into the solution, whereby an added beating effect is secured. If desired, both of the aforementioned means for enhancing the beating action may be employed simultaneously.

10 The drum is also provided with means whereby the various solutions employed in the process may be introduced therein and also with means for removing the solutions during the process as it becomes necessary so to do.

15 In the preferred embodiment of the invention, the drum is mounted on hollow trunnions through at least one of which the various treating agents are introduced as desired, even while the drum is in motion. The outlet is provided at any appropriate place on the drum. The drum is furthermore provided with a door or the like through 20 which the skins to be processed are introduced and the processed skins removed after treatment.

25 In carrying out the process, not less than fifteen dozen skins tanned with chrome tannage, as hereinbefore described, are introduced into the drum and the drum is given a movement of the type hereinbefore described.

30 Usually, tanned skins have a crust condition and contain foreign substances. When this condition is present in the stock it becomes necessary to prepare the stock so as to make it amenable to the treatments which it is to undergo in the process. With this in view, the stock is wet back from the crust condition thereof. As a consequence, the foreign substances are removed 35 from the stock and the latter is so thoroughly wetted that it is in a softened open condition. The wet back treatment depends on the condition of the stock. Satisfactory results are secured when the stock is wet back for approximately 30 minutes in plain water at approximately 100-160° F.

40 After the stock has been wet back as previously described, the liquor is dropped and there is introduced into the drum a composition which incorporates an oil into the stock whereby the fibers thereof are softened. Due to the nature of the composition, any possibility of grease on the surface of the product is eliminated. In the preferred embodiment of this invention, this composition is an aqueous emulsion of a mineral oil. 45 The mineral oil is preferably a white stainless mineral oil which has a viscosity of 60 to 120 at 20° F. when tested in a Saybolt viscosimeter. Any suitable emulsifying agent may be used. Triethanolamine, Twitchell's oil base (mixture of sulphonated olefinic compounds), sulphonated oils, fats, etc. are several illustrative emulsifying agents which may be employed. One emulsifying 50 agent or a plurality thereof may be used.

55 The proportions of the ingredients constituting the emulsion are such as to produce an emulsion having a relatively fine or small particle size. A specific illustrative emulsion which has given satisfactory results consists of 70 parts of mineral oil and 30 parts of Twitchell's oil base (the proportions being by weight) and a sufficient amount of water to give the desired fine particle size. In producing this emulsion, the mineral oil and the emulsifying agents are mixed together and the mixture agitated or stirred until a substantially 60 uniform and homogeneous mixture is obtained. While the agitation is continued, a sufficient quantity of water is added to produce the desired particle size and viscosity. A sufficient quantity of the resulting emulsion is applied to 65 the wet back stock. Though various quantities

70 of emulsion may be introduced into the drum, satisfactory results are secured when an amount of emulsion containing 0.25% to 10% by weight of oil based on the dry weight of the tanned skins is used. The stock is drummed with the emulsion for a sufficient period of time and at a temperature of 140° F. to 160° F. to permit said emulsion to penetrate into the stock. In practice, the desired results have been secured when the wet back stock is drummed with the emulsion for approximately 30 minutes.

75 After drumming the stock with the emulsion as immediately before described, the liquor is dropped and the stock is in condition and ready to receive its body or foundation color which is produced through the medium of dyestuffs. The dyestuffs employed for producing the body or foundation color depend on the tintorial or tone value desired in the final product. Thus, when a dark color is desired, the dyestuff employed in the production of the body or foundation color is one which will produce a dark shade. Likewise, when a light tone effect is desired, a dyestuff which produces a light color is employed in the coloring of the body or foundation color. Though various dyestuffs may be used for producing the foundation color, I prefer those dyestuffs herein referred to as Derma dyestuffs. As illustrative examples of Derma dyestuffs for producing several illustrative colors may be mentioned the following dyestuffs manufactured and sold by the Sandoz Chemical Works of New York:

| Dye                     | Color  | 35 |
|-------------------------|--------|----|
| Dermacarbon B Conc..... | Black. |    |
| Derma blue 2B Conc..... | Blue.  |    |
| Derma brown G Conc..... | Brown. |    |
| Derma brown R Conc..... | Do.    |    |

40 In some instances in order to produce the desired tone of the body or foundation, a mixture of two or more dyestuffs may be used. For example, when a deep black is desired, Dermacarbon B Conc. may be mixed with an appropriate quantity of some other aniline dyestuff, such as, 45 for example, Chloramine Dark Green B Conc., color index #583, or some other green color. The relative proportions of the two dyestuffs depend, of course, on the desired tone to be produced.

50 Though the body or foundation color may be introduced by a single dye application, a better, more level and deeper color is secured when the dyestuff is applied in several applications. Hence, the invention contemplates a plurality or several applications of the dyestuff for producing the body or foundation color.

55 When the dyestuff or dyestuffs employed in the production of the body or foundation color are of the type which requires a mordant, a suitable mordant is incorporated at the same time that the foundation dyestuff or dyestuffs are applied. When the foundation color is produced by several applications of dyestuffs, sufficient mordant is applied in the first stage so as to make it unnecessary to apply it in the second or subsequent 60 applications.

65 Any suitable mordant which does not affect the fibers of the stock but acts only on the dyestuff may be employed. Oxidizable chromium salts have been found especially suitable for this purpose. More satisfactory results are secured when, in conjunction with the oxidizable chromium salts, there is also used a polybasic acid (aliphatic or aromatic), preferably a dicarboxylic acid. As a specific illustrative example of a 70

suitable oxidizable chromium salt may be mentioned sodium bichromate, and as a suitable polybasic acid may be mentioned oxalic, citric, etc. If desired, the chromium salt and the polybasic acid may be mixed together prior to the incorporation in the dye bath. Alternatively, the ingredients constituting the mordant may be added separately to the bath. Thus, the stock may be first stricken with bichromate and then with the selected polybasic acid. The quantity of mordant which may be used depends, of course, on the quantity of dyestuff to be used.

As an illustrative example, a satisfactory deep black foundation color is secured in two applications and when the first application contains the selected mordant in an amount of 0.25% to 10% and the dyestuff is a mixture consisting of 0.5% to 20% Dermacarbon B. Conc. and 0.0625% to 5% Chloramine Dark Green B. Conc. and is drummed at 140° to 160° F. for 45 minutes, and the second application consists of a mixture of 0.25% to 10% Dermacarbon B Conc. and 0.0625% to 5% Chloramine Dark Green B Conc. and is drummed for 30 minutes at 140° to 160° F.

In order to exhaust the dye and to drive the color on to the stock, there is added to the dye bath, preferably in stages, a weakly ionized organic acid, such as, for example, an organic acid which has a dissociation constant not over  $10^{-2}$ . Though formic acid is preferred, other acids having the dissociation constant mentioned, such as, for example, citric, acetic, tartaric, lactic, boric, maleic, may be used. Best results are secured when the acid is added at predetermined intervals in each dye application.

Thus, when the dye application is in two stages, as immediately before described, after the first dye application has been drummed as described, there is added at 10 minute intervals a total of 3 feedings, each containing 0.5% to 20% of formic acid at 135° F. and, after the second dye application and drumming, there is added at 10 minute intervals a total of 3 feedings, each containing 0.25% to 20% formic acid at 135° F. Thereafter the liquor is dropped. The quantity of acid employed is greater than that necessary to exhaust the dyestuffs from the baths and the reason for this will become apparent from the description hereinafter.

After the stock has been given the desired body or foundation color, as previously mentioned, it is subjected to treatments whereby the fibers are rendered in condition so that, upon finishing in accordance with the type of suede desired, the desired properties, such as luster or sheen and silky feel or hand, are secured. This condition of the fibers is secured through a deterioration of the fibers which, in the preferred form of the invention, is secured by a chemical reaction between the reagents upon the surface of and within the fibers and an appropriate reagent or reagents. Prior to or simultaneously with the deterioration of the fibers, the latter are treated so as to either split the tops of the fibers or spread apart the fibers in the fiber bundles, or both. This step is herein referred to as the "fiber separation."

The fiber separation is effected by means of iron hydroxide which is produced in situ in at least the top portions of the surface fibers. According to the invention, there is produced an iron tannate on the surface fibers and a small part of this iron tannate is converted into the hydroxide. Due to the excess acid employed in the dye exhaustion step, there is produced an

acid environment on and in the skins, whereby the precipitation of the iron tannates is retarded.

In practice, after the stock has been colored and the dye liquor dropped, there is introduced into the drum 1% to 20% of tannic acid-bearing materials, such as hematite crystals, fustic crystals, stainless sumac extract, dyewoods, vegetable tanning matter, and the contents maintained at 140° F. Due to the acid condition of the stock resulting from the excess acid employed in the dye exhausting steps, the tannic acid-bearing materials are kept on the surface of the stock. A suitable quantity, such as 0.25% to 20%, of iron (preferably ferrous) salts is then added, whereby an iron tannate is produced. As previously explained, the acid environment retards oxidation of the iron salts, thereby retarding the precipitation of the iron tannates. After being drummed for 15 minutes, the liquor is dropped and the temperature raised to 135° F. and there is added 0.5% to 10% of an alkali or alkaline salt, such as borax, soda, etc. The alkali neutralizes the acid to the point where iron hydroxide is nearly precipitated.

After the addition of the alkali, the materials are drummed for 15 minutes and after dropping the liquor, 0.0625% to 20% of a mildly basic aromatic amine, such as paraphenylenediamine, meta toluylenediamine, etc., is added and drumming continued for one hour, after which the stock is removed from the drum, hoisted up for oxidation and dried in a cool room. The skins are then finished as hereafter described to produce the luster or sheen and silky feel or hand.

When the amine is added, a reaction sets in which deteriorates parts of the fine surface fibers. The alkali has produced such a pH that the mild alkalinity of the amine decomposes some of the iron tannate to produce a bulky precipitate of iron hydroxide. The bulky iron hydroxide separates the fibers, i. e. splits at least a portion of the tops of the fibers or spreads apart the fibers in the fiber bundles, or both, whereby, upon orientation in the finishing operation, the silky finish is secured. However, sufficient unoxidized amine remains on the surface of the fiber to permit oxidation by the air, whereby further deterioration is secured. The deterioration converts the fibers into the desired condition.

In the event the color of the stock is not the exact tone desired, prior to the application of the amine a sufficient quantity of a dyestuff, such as a basic aniline dyestuff in an amount of 1% to 10%, is added to bring the color to the desired tone. When this step is employed, the materials are drummed 30 minutes, the liquor dropped and the amine added as described.

The skins are then finished in accordance with the type of suede finish desired. When a non-croaking suede finish is desired, the skins are finished by drying and dry milling in the manner used in making ordinary suede. When a non-croaking suede finish having a luster and silky feel is desired, the skins are finished as hereafter set forth.

After the skins have been dried in the cool room, they are taken down and put into wet sawdust in which they are left, according to the type of skins, from 4 to 12 hours. The skins are then taken out of the saw-dust and staked and, after they have been staked once, they are blocked with an emery block.

If sheep skins constitute the basis of the stock, they are plushed from the backbone out by a

reel rotating at a speed of from 1600 to 2500 revolutions per minute. After they are plushed, the skins are hand ironed, again staked, and plushed by the plush reel.

5 When kid skins or calf skins are used in the process, after removal from the saw-dust, they are staked and plushed like the sheep skins and then put into a drying drum and dry-milled from 6 to 12 hours. After removal from the drying 10 drum, the skins are successively toggled, staked, plushed, ironed, staked, and plushed again.

In order to more fully explain the invention, there is hereafter set forth an illustrative example for producing a deep black product. The 15 portions are by weight based on the dry weight of the tanned skins in crusted condition.

The desired number of tanned skins of the selected stock is introduced into the drum and wet back for 30 minutes in plain water at 160° F. 20 After dropping the liquor, there is added a sufficient quantity of the mineral oil emulsion so as to provide 3% of the mineral oil. After drumming for 30 minutes, the liquor is dropped and there is added a previously prepared mixture 25 containing 4% of Dermacarbon Black B Conc. and 0.75% of Chloramine Dark Green B Conc. Either simultaneously with or subsequently to the introduction of the dyestuffs, there is added 3% of the bichromate polybasic acid mordant. After 30 drumming for 45 minutes at 160° F., there is added in three feedings at 10 minute intervals at 135° F. 1.25% of formic acid for each feeding. Then there is added a mixture containing 4% of Dermacarbon Black B Conc. and 0.75% of 35 Chloramine Dark Green B Conc. After drumming for 30 minutes of 160° F., there is added in three feedings at 10 minute intervals 1.25% of formic acid for each feeding. The liquor is then dropped and a mixture of 5% of hematite crystals, 1.50% of fustic crystals and 1.50% of stain- 40 less sumac extract at 145° F. is added and the mass drummed for 30 minutes at 145° F. The mass is then stricken with 5% of copperas and 1% of iron nitrate (ferric sulphate, ferric sulphate nitrate, basic ferric sulphate nitrate) and 45 drummed for 15 minutes, after which the liquor is dropped. The temperature is brought back to 135° F. and 2% of borax is added. After drumming for 15 minutes, there is added 4% of basic aniline dyestuffs. After drumming for 30 minutes, the liquor is dropped and 1% of paraphenylene diamine is added. After drumming for 1 hour, the skins are removed from the drum, horsed up for oxidation, and dried in a cool room. 50 The skins are then finished as previously described.

The product resulting from the specific procedure hereinbefore set forth is a deep black soft leather having a non-croaking suede finish characterized by a luster or sheen and silky feel or hand comparable to genuine French antelope. Obviously, by using appropriate dyestuffs, other colored products can be produced. By utilizing the finishing procedure normally used in the production of regular suede and varying the times and concentrations of the specific procedure hereinbefore set forth, as will be obvious to a person skilled in the art, a non-croaking suede can be obtained.

70 Since it is obvious that various changes and modifications may be made in the above description without departing from the nature and spirit thereof, this invention is not restricted thereto except as set forth in the appended claims.

75 I claim:

1. In a method of producing a colored suede finish on skins containing chrome tannage, the steps which comprise dyeing a plurality of the selected skins, separating the fibers by chemically producing a bulky deposit on and between the fibers on the surface of the dyed skins, and subjecting the skins to a finishing treatment. 5

2. In a method of producing a colored suede finish on skins containing chrome tannage, the steps which comprise dyeing a plurality of the selected skins, forming iron hydroxide in and on at least the top portions of the fibers on the surface of the dyed skins, by causing an iron compound in the presence of alkaline compounds to react with an aromatic amine, and subjecting 10 the skins to a finishing treatment. 15

3. In a method of producing a colored suede finish on skins containing chrome tannage, the steps which comprise dyeing a plurality of the selected skins, forming an iron compound in and on at least the top portions of the fibers on the surface of the dyed skins, again dyeing the skins to produce the tinctorial effect desired in the final product, causing said iron compound in the presence of alkaline compounds to react with an aromatic amine, and subjecting 20 the skins to a finishing treatment. 25

4. In a method of producing a colored suede finish on skins containing chrome tannage, the steps which comprise treating a plurality of wet back skins with an aqueous mineral oil emulsion, dyeing said skins, separating the fibers by chemically producing a bulky deposit on and between the fibers on the surface of the dyed skins, and subjecting the skins to a finishing treatment. 30

5. In a method of producing a colored suede finish on skins containing chrome tannage, the steps which comprise treating a plurality of wet back skins with an aqueous mineral oil emulsion, 40 dyeing said skins, forming iron hydroxide in and on at least the top portions of the fibers on the surface of the dyed skins by causing an iron compound in the presence of alkaline compounds to react with an aromatic amine, and subjecting the skins to a finishing treatment. 45

6. In a method of producing a colored suede finish on skins containing chrome tannage, the steps which comprise treating a plurality of wet back skins with an aqueous mineral oil emulsion, dyeing said skins, forming an iron compound in 50 and on at least the top portions of the fibers on the surface of the dyed skins, again dyeing the skins to produce the tinctorial effect desired in the final product, causing said iron compound in the presence of alkaline compounds to react 55 with an aromatic amine, and subjecting the skins to a finishing treatment.

7. In a method of producing a colored suede finish on skins containing chrome tannage, the steps which comprise dyeing a plurality of the selected skins in the presence of an amount of a weakly ionized organic acid in excess of that required to exhaust the dye whereby an acid environment is produced in the skins, forming iron tannate in and on at least the top portions of the 65 surface fibers, neutralizing the acid with an alkaline compound to a point where a portion of the iron tannate is nearly precipitated as iron hydroxide, applying an aromatic amine in an amount in excess of that required to precipitate 70 the iron hydroxide, permitting the excess amine to oxidize, and subjecting the skins to a finishing treatment.

8. In a method of producing a colored suede finish on skins containing chrome tannage, the 75

5 steps which comprise dyeing a plurality of the selected skins containing chrome tannage in the presence of an amount of an organic acid having a dissociation constant not over  $10^{-2}$  in excess of that required to exhaust the dye whereby an acid environment is produced in the skins, forming iron tannate in and on at least the top portions of the surface fibers, neutralizing the acid with an alkaline compound to a point where a 10 portion of the iron tannate is nearly precipitated as iron hydroxide, applying an aromatic amine in an amount in excess of that required to precipitate the iron hydroxide, permitting the excess amine to oxidize, and subjecting the skins 15 to a finishing treatment.

9. In a method of producing a colored suede finish on skins containing chrome tannage, the steps which comprise dyeing a plurality of the selected skins containing chrome tannage in the 20 presence of an amount of an organic acid having a dissociation constant not over  $10^{-2}$  in excess of that required to exhaust the dye whereby an acid environment is produced in the skins, forming iron tannate in and on at least the top 25 portions of the surface fibers, neutralizing the acid with an alkaline compound to a point where a portion of the iron tannate is nearly precipitated as iron hydroxide, again dyeing the skins to produce the tinctorial effect desired in the product, 30 applying an aromatic amine in an amount in excess of that required to precipitate the iron hydroxide, permitting the excess amine to oxidize, and subjecting the skins to a finishing treatment.

10. In a method of producing a colored suede 35 finish on skins containing chrome tannage, the steps which comprise treating a plurality of wet back skins containing chrome tannage with an aqueous mineral oil emulsion, dyeing the skins in the presence of an amount of a weakly ionized 40 organic acid in excess of that required to exhaust the dye whereby an acid environment is produced in the skins, treating the dyed skins with a composition containing tannic acid-bearing materials, striking the skins with an iron salt, neutralizing 45 the acid to a point where some iron hydroxide is nearly precipitated, adding an aromatic amine in an amount in excess of that required to precipitate the iron hydroxide, permitting the excess amine to oxidize, drying the skins, and finally 50 subjecting the skins to a finishing treatment.

11. In a method of producing a colored suede finish on skins containing chrome tannage, the steps which comprise treating a plurality of wet back skins containing chrome tannage with an 55 aqueous mineral oil emulsion, dyeing the skins in a dye bath containing an organic acid having a dissociation constant not over  $10^{-2}$  and in an amount in excess of that required to exhaust the dye whereby an acid environment is produced in the skins, treating the dyed skins with a composition containing tannic acid-bearing materials, striking the skins with an iron compound, applying an alkaline salt in an amount to 60 produce a condition where some iron hydroxide is nearly precipitated, again dyeing the skins to produce the tinctorial effect desired in the final product, adding an aromatic amine in an amount in excess of that required to precipitate the iron hydroxide, permitting the excess amine to oxidize, drying the skins, and finally subjecting the skins to a finishing treatment.

12. In a method of producing a colored suede finish on skins containing chrome tannage, the steps which comprise treating a plurality of wet 75 back skins containing chrome tannage with an

aqueous mineral oil emulsion, dyeing the skins in a dye bath containing a dyestuff requiring a mordant and in the presence of a mordant, adding to the dye bath an organic acid having a dissociation constant not over  $10^{-2}$  and in an amount in excess of that required to exhaust the dye whereby an acid environment is produced in the skins, treating the dyed skins with a composition containing tannic acid-bearing materials, striking the skins with an iron salt, neutralizing the acid with an alkaline compound to a point where some iron hydroxide is nearly precipitated, adding an aromatic amine in an amount in excess of that required to precipitate the iron hydroxide, permitting the excess amine to oxidize, drying the skins, and finally subjecting the skins to a finishing treatment.

13. In a method of producing a colored suede finish on skins containing chrome tannage, the steps which comprise treating a plurality of wet back skins containing chrome tannage with an aqueous mineral oil emulsion, dyeing the skins in a dye bath with a dyestuff requiring a mordant and in the presence of a bichromate polybasic acid mordant, adding to the dye bath an organic acid having a dissociation constant not over  $10^{-2}$ , adding an additional dyestuff to the dye bath, again adding said organic acid, the total quantity of organic acid added being in excess of that required to exhaust the dye whereby an acid environment is produced in the skins, treating the dyed skins with a composition containing tannic acid-bearing materials, striking the skins with an iron salt, neutralizing the acid with an alkaline compound to a point where some iron hydroxide is nearly precipitated, adding an aromatic amine in an amount in excess of that required to precipitate the iron hydroxide, permitting the excess amine to oxidize, drying the skins, and finally subjecting the skins to a finishing treatment.

14. In a method of producing a colored suede finish on skins containing chrome tannage, the steps which comprise treating a plurality of wet back skins containing chrome tannage with an aqueous mineral oil emulsion, dyeing the skins in a dye bath containing a dyestuff requiring a mordant and in the presence of a bichromate polybasic acid mordant, intermittently adding to the dye bath at predetermined intervals an organic acid having a dissociation constant not over  $10^{-2}$ , adding an additional dyestuff to the dye bath, again intermittently adding said organic acid at predetermined intervals, the total quantity of organic acid added being in excess of that required to exhaust the dye whereby an acid environment is produced in the skins, treating the dyed skins with a composition containing tannic acid-bearing materials, striking the skins with an iron salt, neutralizing the acid with an alkaline compound to a point where some iron hydroxide is nearly precipitated, adding an aromatic amine in an amount in excess of that required to precipitate the iron hydroxide, permitting the excess amine to oxidize, drying the skins, and finally subjecting the skins to a finishing treatment.

15. In a method of producing a colored suede finish on skins containing chrome tannage, the steps which comprise treating a plurality of wet back skins containing chrome tannage with an aqueous mineral oil emulsion, dyeing the skins in a dye bath containing a dyestuff requiring a mordant and in the presence of a bichromate polybasic acid mordant, intermittently adding to

- the dye bath at predetermined intervals an organic acid having a dissociation constant not over  $10^{-2}$ , adding an additional dyestuff to the dye bath, again intermittently adding said organic acid at predetermined intervals, the total quantity of organic acid added being in excess of that required to exhaust the dye whereby an acid environment is produced in the skins, treating the dyed skins with a composition containing 5 tannic acid-bearing materials, striking the skins with an iron salt, neutralizing the acid with an alkaline compound to a point where some iron hydroxide is nearly precipitated, dyeing the skins to produce the tinctorial effect desired in the 10 final product, adding an aromatic amine in an amount in excess of that required to precipitate the iron hydroxide, permitting the excess amine to oxidize, drying the skins, and finally subjecting the skins to a finishing treatment.
- 15 20. In a method of producing a colored suede finish on skins containing chrome tannage, the steps which comprise dyeing a plurality of the selected skins in a drum, separating the fibers by chemically producing a bulky deposit on and 25 between the fibers on the surface of the dyed skins while in said drum, and thereafter removing the skins from the drum and subjecting them to a finishing treatment.
- 25 30. In a method of producing a colored suede finish on skins containing chrome tannage, the steps which comprise dyeing a plurality of the selected skins, forming iron hydroxide in and on at least the top portions of the fibers on the surface of the dyed skins by causing an iron compound in the presence of alkaline compounds to react with an aromatic amine, each of the previous steps being performed in a drum whereby a drumming action is secured, and after removing the skins from said drum subjecting the skins 35 to a finishing treatment.
- 35 40. In a method of producing a colored suede finish on skins containing chrome tannage, the steps which comprise dyeing a plurality of the selected skins in the presence of an amount of weakly ionized organic acid in excess of that required to exhaust the dye whereby an acid environment is produced in the skins, forming iron tannate in and on at least the top portions of the surface fibers, neutralizing the acid to a point 45 where a portion of the iron hydroxide is nearly precipitated as iron hydroxide, applying an aromatic amine in excess of that required to precipitate the iron hydroxide, each of the previous steps being performed in a drum with a drumming action, removing the skins from the drum, permitting the excess amine to oxidize, and finally subjecting the skins to a finishing treatment.
- 50 55. In a method of producing a colored suede finish on skins containing chrome tannage, the steps which comprise wetting back a plurality of skins containing chrome tannage for 30 minutes in plain water at from 100° F. to 160° F. in a rotating drum, dropping the liquor, adding a sufficient quantity of an aqueous mineral oil emulsion to provide approximately 0.25% to 10% of mineral oil, drumming the skins and mineral oil emulsion for 30 minutes at 140° F. to 160° F., dropping the liquor, adding the selected dyestuff, incorporating a sufficient quantity of a bichromate 60 polybasic acid mordant to act on the dyestuff employed in the process, drumming the skins and dyestuffs for approximately 45 minutes at 140° F. to 160° F., adding formic acid in three feedings at 10 minute intervals at 135° F., each feeding containing 0.5% to 20% formic acid, adding an additional dyestuff, drumming for 30 minutes at 160° F., adding formic acid in three feedings at 10 minutes intervals, each feeding containing 1.25% of formic acid, dropping the liquor, adding a mixture of tannic acid-bearing materials containing 5% of hematite crystals, 1.5% of fustic 65 70 75
- additional dyestuff, drumming for 30 minutes at 140° F. to 160° F., adding formic acid in three feedings at 10 minute intervals at 135° F., each feeding containing 0.25% to 20% formic acid, dropping the liquor, adding 1% to 20% of tannic acid-bearing materials, drumming the mass for 30 minutes at 145° F., striking with 0.25% to 20% of an iron salt, drumming for 15 minutes, dropping the liquor, bringing back the temperature to 135° F., adding 0.5% to 10% of an alkaline compound, drumming for 15 minutes, adding 0.625% to 20% of an aromatic amine, drumming for 1 hour, removing the skins from the drum, horsing up said skins to permit the amine to oxidize, drying said skins in a cool room, and finally subjecting the skins to a finishing operation.
- 10 15 20. In a method of producing a colored suede finish on skins containing chrome tannage, the steps which comprise wetting back a plurality of skins containing chrome tannage for 30 minutes in plain water at from 100° F. to 160° F. in a rotating drum, dropping the liquor, adding a sufficient quantity of an aqueous mineral oil emulsion to provide approximately 0.25% to 10% of mineral oil, drumming the skins and mineral oil emulsion for 30 minutes at 140° F. to 160° F., dropping the liquor, adding the selected dyestuff, incorporating a sufficient quantity of a bichromate 25 polybasic acid mordant to act on the dyestuff employed in the process, drumming the skins and dyestuffs for approximately 45 minutes at 140° F. to 160° F., adding formic acid in three feedings at 10 minute intervals at 135° F., each feeding containing 0.5% to 20% formic acid, adding an additional dyestuff, drumming for 30 minutes at 140° F. to 160° F., adding formic acid in three feedings at 10 minute intervals at 135° F., each feeding containing 0.25% to 25% formic acid, dropping the liquor, adding 1% to 20% of tannic acid-bearing materials, drumming the mass for 30 minutes at 145° F., striking with 0.25% to 20% of an iron salt, drumming for 15 minutes, dropping the liquor, bringing back the temperature to 135° F., adding 0.5% to 10% of an alkaline compound, drumming for 15 minutes, adding 1% to 10% of a basic aniline dyestuff, drumming for 30 minutes, dropping the liquor, adding 0.625% to 20% of an aromatic amine, drumming for 1 hour, removing the skins from the drum, horsing up said skins to permit the amine to oxidize, drying said skins in a cool room, and finally subjecting the skins to a finishing operation.
- 30 35 40. In a method of producing a colored suede finish on skins containing chrome tannage, the steps which comprise wetting back a plurality of skins containing chrome tannage for 30 minutes in plain water at 160° F. in a rotating drum, dropping the liquor, adding a sufficient quantity of an aqueous mineral oil emulsion to provide approximately 3% of mineral oil, drumming the skins and mineral oil emulsion for 30 minutes, dropping the liquor and then adding a selected dyestuff, incorporating 3% of a bichromate polybasic acid mordant in the dye bath, drumming the skins and dye bath for approximately 45 minutes at 160° F., adding formic acid in three feedings at 10 minute intervals at 135° F., each feeding containing 1.25% of formic acid, adding an additional dyestuff, drumming for 30 minutes at 160° F., adding formic acid in three feedings at 10 minutes intervals, each feeding containing 1.25% of formic acid, dropping the liquor, adding a mixture of tannic acid-bearing materials containing 5% of hematite crystals, 1.5% of fustic 45 50 55 60 65 70 75
21. In a method of producing a colored suede finish on skins containing chrome tannage, the steps which comprise wetting back a plurality of skins containing chrome tannage for 30 minutes in plain water at 160° F. in a rotating drum, dropping the liquor, adding a sufficient quantity of an aqueous mineral oil emulsion to provide approximately 3% of mineral oil, drumming the skins and mineral oil emulsion for 30 minutes, dropping the liquor and then adding a selected dyestuff, incorporating 3% of a bichromate polybasic acid mordant in the dye bath, drumming the skins and dye bath for approximately 45 minutes at 160° F., adding formic acid in three feedings at 10 minute intervals at 135° F., each feeding containing 1.25% of formic acid, adding an additional dyestuff, drumming for 30 minutes at 160° F., adding formic acid in three feedings at 10 minutes intervals, each feeding containing 1.25% of formic acid, dropping the liquor, adding a mixture of tannic acid-bearing materials containing 5% of hematite crystals, 1.5% of fustic 70 75

- crystals and 1.5% of stainless sumac extract at 145° F., drumming the mass for 30 minutes at 145° F., striking with 5% of copperas and 1% of iron nitrate, drumming for 15 minutes, dropping the liquor, bringing back the temperature to 135° F., adding 2% of borax, drumming for 15 minutes, adding 4% of a basic aniline dyestuff, drumming for 30 minutes, dropping the liquor, adding 1% of paraphenyl diamine, drumming for 1 hour, 5 removing the skins from the drum, horsing up said skins for oxidation, drying said skins in a cool room, and finally subjecting the skins to a finishing treatment.
22. In a method of producing a colored suede 15 finish on skins containing chrome tannage as set forth in claim 7, a finishing treatment which comprises covering the previously prepared and dried skins with wet saw-dust, removing the saw-dust, staking the skins, blocking the staked skins 20 with an emery block, plushing the skins, ironing, and again staking and plushing the skins.
23. In a method of producing a colored suede 25 finish on sheep skins as set forth in claim 7, the finishing treatment which comprises covering the previously prepared skins with wet saw-dust for 4 to 12 hours, removing the skins from the saw-dust, staking said skins, blocking said skins with an emery block, plushing said skins from the backbone out by a plushing reel rotating at from 1600 to 2500 R. P. M., thereafter ironing said 30 skins, and then again staking and plushing said skins.
24. In a method of producing a colored suede 35 finish on kid or calf skins as set forth in claim 7, the finishing treatment which comprises covering the previously prepared skins with wet saw-dust, removing the skins from the saw-dust, staking said skins, blocking said skins with an emery block, plushing said skins from the backbone, out by a plushing reel rotating at from 1600 to 2500 40 R. P. M., dry milling said skins in a drum for 6 to 12 hours, and thereafter successively subjecting the skins to toggling, staking, plushing, ironing, staking and plushing operations.
25. In a method of producing a colored suede 45 finish on skins containing chrome tannage, the steps which comprise dyeing a plurality of the selected skins, forming iron hydroxide in and on at least the top portions of the fibers on the surface of the dyed skins by causing an iron compound in the presence of alkaline compounds to react with an aromatic amine, the quantity of amine being in excess of the amount necessary to produce said iron hydroxide, causing the excess amine to oxidize on the fibers, and subjecting the skins to a finishing treatment.
26. In a method of producing a colored suede 50 finish on skins containing chrome tannage, the steps which comprise treating a plurality of wet back skins with an aqueous mineral oil emulsion, dyeing said skins, forming iron hydroxide in and on at least the top portions of the fibers on the surface of the dyed skins by causing an iron compound in the presence of alkaline compounds to react with an aromatic amine, the quantity of amine being in excess of the amount necessary to produce said iron hydroxide, causing the excess amine to oxidize on the fibers, and subjecting the skins to a finishing treatment.
27. In a method of producing a colored suede 55 finish on skins containing chrome tannage, the steps which comprise treating a plurality of wet back skins with an aqueous mineral oil emulsion, dyeing said skins, forming iron hydroxide in and on at least the top portions of the fibers on the surface of the dyed skins by causing an iron compound in the presence of alkaline compounds to react with an aromatic amine, each of the previous steps being performed in a drum whereby a drumming action is secured, removing the skins from said drum, and subjecting said skins to a finishing treatment.
28. In a method of producing a colored suede 60 finish on skins containing chrome tannage, the steps which comprise treating a plurality of wet back skins containing chrome tannage with an aqueous mineral oil emulsion, dyeing the skins in the presence of an amount of a weakly ionized organic acid in excess of that required to exhaust the dye whereby an acid environment is produced in the skins, treating the dyed skins with a composition containing tannic acid-bearing materials, striking the skins with an iron salt, neutralizing the acid to a point where some iron hydroxide is nearly precipitated, adding an aromatic amine in an amount in excess of that required to precipitate the iron hydroxide, permitting the excess amine to oxidize, each of the previous steps being performed in a drum whereby a drumming action is secured, removing the skins from said drum, drying said skins, and finally subjecting the skins to a finishing treatment.
29. In a method of producing a colored suede 65 finish on skins containing chrome tannage, the steps which comprise dyeing a plurality of the selected skins, separating the fibers by chemically producing a bulky deposit on and between the fibers on the surface of the dyed skins, each of the steps being performed at a temperature of from 100° F. to 160° F. in a drum whereby a drumming action is secured, removing the skins from the drum, and subjecting the skins to a finishing treatment.
30. In a method of producing a colored suede 70 finish on skins containing chrome tannage, the steps which comprise dyeing a plurality of the selected skins, forming iron hydroxide in and on at least the top portions of the fibers on the surface of the dyed skins by causing an iron compound in the presence of alkaline compounds to react with an aromatic amine, each of the previous steps being performed at a temperature of from 100° F. to 160° F. in a drum whereby a drumming action is secured, removing the skins from said drum, and subjecting said skins to a finishing treatment.
31. In a method of producing a colored suede 75 finish on skins containing chrome tannage, the steps which comprise treating a plurality of wet back skins with an aqueous mineral oil emulsion, dyeing said skins, forming iron hydroxide in and on at least the top portions of the fibers on the surface of the dyed skins by causing an iron compound in the presence of alkaline compounds to react with an aromatic amine, each of the preceding steps being performed at a temperature of from 100° F. to 160° F. in a drum whereby a drumming action is secured, removing the skins from the drum, and subjecting the skins to a finishing treatment.

CERTIFICATE OF CORRECTION.

Patent No. 2,204,262.

June 11, 1940.

ERNEST RUDOLF STERN.

It is hereby certified that error appears in the printed specification of the above numbered patent requiring correction as follows: Page 4, first column, line 36, for "of" read --at--; page 6, first column, line 69, claim 19, for "ncorporating" read --incorporating--; same page, second column, line 38, claim 20, for "0.25% to 25%" read --0.25% to 20%--; line 47, same claim, for "dopping" read --dropping--; line 72, claim 21, for "minutes" read --minute--; and that the said Letters Patent should be read with this correction therein that the same may conform to the record of the case in the Patent Office.

Signed and sealed this 30th day of July, A. D. 1940.

(Seal)

Henry Van Arsdale,  
Acting Commissioner of Patents.